

# UNITED STATES PATENT OFFICE.

HORACE CAMPBELL HALL, OF DERBY, ENGLAND, ASSIGNOR TO ROLLS-ROYCE LIMITED, OF DERBY, ENGLAND, A COMPANY OF GREAT BRITAIN.

## ALUMINUM ALLOY.

1,418,303.

Specification of Letters Patent. Patented June 6, 1922.

No Drawing.

Application filed February 18, 1921. Serial No. 446,115.

To all whom it may concern:

Be it known that I, HORACE CAMPBELL HALL, of Derby, England, have invented certain new and useful Improvements in 5 Aluminum Alloys, of which the following is a specification.

This invention consists of improved aluminum alloys. According to this invention an alloy is made consisting of—

10 Copper about .1% to any amount below 3%.

Titanium about .1% to about 2%.

Zinc about 6% to about 16%.

15 Iron (present as an impurity of commercial aluminum) preferably not exceeding .6%.

Silicon (present as an impurity of commercial aluminum) preferably not exceeding .4%.

20 Other elements (impurities) preferably not exceeding .4%.

Aluminum remainder.

The alloy can be made as follows:—

25 A copper-titanium aluminum alloy should be made in the first instance consisting of—

Copper about 32%.

Titanium about 7.5%.

Aluminum about 59%.

30 Other elements (impurities) preferably not exceeding 1.5%.

In the above the quantities of titanium and aluminum may be varied about 2% above or below the percentages stated. Further a slightly higher percentage of 35 copper may be used dependent on the ultimate properties required.

The alloy so made is then introduced in the form of suitable sized pieces or granules into a bath of molten commercial aluminum 40 in which it will readily dissolve. The zinc should then be added but it is preferable to retain a small proportion, say 1% thereof to be added later as hereinafter explained.

If it is desired to increase the ratio of 45 copper to titanium it should be done by the addition of a copper aluminum alloy to the ultimate bath simultaneously with the primary alloy.

The alloy is improved by the substitution 50 for not exceeding 3% of the aluminum, of antimony and/or magnesium not exceeding in respect of either about 1.5%.

If antimony or magnesium or both are required these should preferably be added 55 to the final bath of metal together with the

small percentage of the zinc about 5 minutes before casting.

The introduction of the small quantity of zinc retained as aforesaid at the stage prescribed augments the clearing action of the 60 antimony and magnesium and even by itself makes the metal more fluid.

Alloys made according to this invention of the composition specified above are found to give the following advantages over 65 aluminum alloys heretofore in use:—

1. Increased fluidity in the molten condition.

2. A reduced tendency to crack in the mould during solidification.

3. An absence of gas cavities, resulting in sounder and finer grained castings.

4. An improvement in mechanical test results, including a raising of the yield point, and an increase in ductility.

5. A reduction in the co-efficient of heat expansion of the resulting alloy.

What I claim as my invention and desire to secure by Letters Patent of the United States is:—

1. An alloy, comprising 1 to 3% copper; 1 to 2% titanium; 6 to 16% zinc; and impurities contained in commercial aluminum, not exceeding 1% in the aggregate; the remainder consisting mostly of aluminum.

2. An alloy, comprising 1 to 3% copper; 1 to 2% titanium; 6 to 16% zinc; magnesium, not exceeding 1.5%; and impurities contained in commercial aluminum, not exceeding 1% in the aggregate; the remainder 90 consisting mostly of aluminum.

3. An alloy, comprising 1 to 3% copper; 1 to 2% titanium; 6 to 16% zinc; magnesium, and antimony, not exceeding 1.5% of each; and impurities contained in commercial aluminum, not exceeding 1% in the aggregate; the remainder consisting mostly of aluminum.

4. The process of forming an alloy, comprising the steps of first forming a copper-titanium-aluminum alloy; introducing such alloy in particles of suitable size into a bath of molten commercial aluminum to be dissolved therein; and then adding zinc to the resultant mixture.

5. The process of forming an alloy, comprising the steps of first forming a copper-titanium-aluminum alloy; introducing such alloy in particles of suitable size into a bath of molten commercial aluminum to be dis- 110

solved therein; then adding zinc; and then adding magnesium to the resultant mixture.

6. The process of forming an alloy, comprising the steps of first forming a copper-titanium-aluminum alloy; introducing such alloy in particles of suitable size into a bath of molten commercial aluminum to be dissolved therein; then adding zinc; and then

adding magnesium and antimony to the resultant mixture. 10

In witness whereof I have signed this specification in the presence of two witnesses.

HORACE CAMPBELL HALL.

Witnesses:

NORMAN HAY WALKER,  
VIOLET MAUD MASTERS.